

Apr. 3, 1923.

1,450,699

A. C. MORSE ET AL

PROCESS FOR SEAMLESS TUBE DRAWING

Filed Sept. 13, 1921



*Fig. 1.*



*Fig. 2.*

Inventors  
Alvors C. Morse  
and  
Henry Richard Lewis Jr.  
John N. Goss  
By their Attorney

## UNITED STATES PATENT OFFICE.

ALONZO CLAY MORSE AND HARRY RICHARD LEWIS, JR., OF SHELBY, OHIO.

## PROCESS FOR SEAMLESS-TUBE DRAWING.

Application filed September 13, 1921. Serial No. 500,414.

*To all whom it may concern:*

Be it known that ALONZO CLAY MORSE and HARRY RICHARD LEWIS, Jr., citizens of the United States of America, residing at 5 Shelby, in the county of Richland and State of Ohio, have invented certain new and useful Improvements in Processes for Seamless-Tube Drawing, of which the following is a specification.

10 This invention relates to an improvement in the process of seamless tube drawing, wherein through a definite step of heat-treatment, the qualities and capabilities of the material for the specific purpose outlined, are materially increased.

In the ordinary method of tube making the billets are pierced while hot and rolled over plugs while hot, then pointed and pickled and cold drawn through a die over 20 a mandrel. The product is then annealed in a furnace, at from thirteen hundred to fifteen hundred degrees F., and cooled. The pickling step is then repeated, and the material cold drawn over a mandrel. The operations from the annealing step being successively repeated until the tubing has reached the desired size.

The improved step to be introduced into the process outlined above, is that of heat-treatment of the material to a point just 30 above the critical point of the particular material being used and in accordance with the properties desired and quenching the heated material in a proper cooling medium. This particular heat-treatment step results in a tempering—so called—of the grain of the material, with the obvious advantage of a much greater tensile strength for the same ductility; a more uniform and better grain 35 structure; presents a tubing capable of better and more perfect machining; and produces less scale in annealing, hence requiring less acid and time in pickling and cold drawing.

40 After the tube is quenched, the temper is drawn by reheating to a temperature below that of the temperature at which quenching is had, this drawing temperature, say of a minimum of 300° F. being determined by 45 the required characteristics of the final product, that is the required degree of softness, ductility or other physical properties of the tube desired. The tube is then allowed to cool and the ordinary operations of making

seamless drawn tubing repeated, until the 55 desired size of tube is obtained.

The use of this additional heat-treatment step is not confined to any particular period of the complete process, as the usual process can be followed to any desired size of 60 cold drawn tube, the improved heat-treatment step carried out, and the original or other steps employed to complete the tube formation.

Of course it is to be understood that the 65 heat-treatment step of the process is limited in heat-degree or critical point, by the character of the material being employed, that is its carbon proportion, or nature of alloy, and that, therefore, there can be no specific 70 heat limit referred to for the new step.

The accompanying drawing illustrates a magnified section of material, that in Fig. 1 showing the fiber construction of the material following the old and usual process; and 75 Fig. 2 showing the same material following the introduction of the heat-treatment step of the new process.

The heat treatment, or grain refining step, 80 may, of course, be used in a particular operation as often as desired or necessary; can be performed at any time, after any heating process of the material; or may be carried out after several steps or treatments of the tube. In other words there is no practical 85 limitation to the application of the new step.

Fig. 2 of the drawings, in comparison with Fig. 1, clearly indicates the fiber change incident to the use of the new step, and the advantages of the resultant fiber arrangement will be obvious to one skilled in tube-drawing processes.

The tube resultant from the use of the new step is essentially stronger, that is of greater tensile strength, than the tube resultant from the old or usual process. Therefore, the tube under the new process can be made of much lighter gage, and will necessarily be more perfect, as it is not necessary to heat the tube to such a high degree of heat in annealing, 100 as was required in the old process. The possibility of lower annealing heat prevents a large proportion of otherwise usual scale accumulation, and also avoids the possibility of burning the fibers of the material. As a direct result of these conditions, the material can be worked at a much lower heat 105 and much longer.

The close knitting of the fibers of the material resultant directly from the new step of the process, permits a much better machining of the finished tube than is possible under the old process.

Of course the ordinary tempering of steel has been heretofore known, but the present process is limited to the application to a so called tempering step, involved in a particular heat-treatment and quenching of the material used in process of making, to thereby provide a more perfect product, one stronger and capable of finer drawing, and one requiring less operations to perfect, and providing a better finished article, primarily incident to the permitted use of a lower annealing temperature.

Having thus described the invention, what we claim as new, is:

20. 1. A step in the process of seamless tube drawing, consisting in a refinement of the grain of the metal by heat-treatment to a predetermined degree and then quenching.
21. 2. A step in the process of seamless tube drawing, consisting in heating the material to the upper critical point and quenching intermediate the drawing steps.
22. 3. A step in the process of seamless tube drawing, including heat treatment and quenching prior to the annealing step.
23. 4. A step in the process of seamless tube drawing, consisting in annealing the material, reheating to the upper critical point, quenching, and then tempering for additionally refining the grain of the metal over that of the annealing treatment.
24. 5. A step in the process of seamless tube drawing including heat treatment and quenching immediately following any independent heating step of the usual process.
25. 6. That step in a seamless tube drawing process consisting in heating the material to a temperature just above the critical point and then quenching.

7. An independent step in the process of 45 seamless tube drawing, consisting in heating the metal to a degree to produce refinement of the grain, then quenching, and finally subjecting the metal to a drawing temperature less than the previous heat degree. 50

8. A process consisting in cold drawing a tube and subjecting the tube to an annealing step, a quenching step, and a tempering step, before or between any of the drawing steps.

9. A step in a cold drawing tube process 55 directed toward extreme refinement of the grain of the metal, consisting in heating the material to the critical point and quenching in a cooling medium and thereafter annealing.

10. A process for drawing seamless tubing consisting of piercing and drawing said billet over a plug in a heated state, then pointing same, then heating same to a temperature just above the critical point, then quenching same in a cooling medium; then re-heating to a temperature below the upper critical point depending on the character or quality of the steel desired and then allowing same to cool and repeating the usual operations 70 until the size required is produced.

11. A process for drawing seamless tubing consisting of piercing a billet and drawing said billet over a plug in a heated state, then pointing same, then heating same to a temperature just above the critical point, then quenching same in a cooling medium, then reheating same to a temperature between 300° F. and the upper critical point, depending on the character or quality of the tube desired, and then allowing same to cool and repeating the usual operation of drawing the tube until the tube is finished to the size desired. 75

In testimony whereof we affix our signatures.

ALONZO CLAY MORSE.

HARRY RICHARD LEWIS, JR.